

# UNITED STATES PATENT OFFICE.

FRANZ ANDRÁSEK AND JOSEF DRECHSLER, OF ZILINA, CZECHOSLOVAKIA.

## PROCESS OF PRODUCING JOINT-MAKING PACKING.

No Drawing.

Application filed November 2, 1922. Serial No. 598,696.

*To all whom it may concern:*

Be it known that we, FRANZ ANDRÁSEK and JOSEF DRECHSLER, citizens of the Republic of Czechoslovakia, residing at Zilina, 5 Czechoslovakia, have invented certain Processes of Producing Joint-Making Packing, of which the following is a specification.

This invention relates to a joint-making packing of the kind composed of a powder of soft metal which is mixed with asbestos, graphite and a viscous lubricant, and more particularly to a method of comminuting the metal, its object being to produce uniform metal particles capable of rendering 10 the packing very elastic and durable. This object is achieved according to the invention by pouring the molten metal into a bag of refractory sieve material and rubbing said bag against a warm plate until the greater 15 part of the metal has passed through in the form of grains or as a powder.

The metal may consist of lead or an alloy

of such. The bag may be made out of a muslin of suitable mesh which is rendered refractory in known manner, for instance by 25 impregnation with alum and ammonium sulphate.

We claim:

1. A method of comminuting soft metal for use with joint-making packing, consisting in pouring the molten metal into a bag of refractory sieve material, and rubbing the bag against a warm plate until the greater part of the metal has passed through in the form of a powder. 30

2. A method of comminuting soft metal for use with joint-making packing, consisting in pouring the molten metal into an impregnated, refractory muslin bag, and rubbing said bag against a warm plate until 35 the greater part of the metal has passed through in the form of a powder. 40

FRANZ ANDRÁSEK.  
JOSEF DRECHSLER.